

W. H. UNDERWOOD.  
METALLIC YARN AND FABRIC.  
APPLICATION FILED NOV. 12, 1910.

1,012,031.

Patented Dec. 19, 1911.

*Fig. 1*



*Fig. 2*



*Fig. 3*



*Fig. 4*



*Fig. 5*



*Fig. 6*



*Fig. 7*



Witnesses:  
A. C. Parham  
M. M. Riemann

W. H. Underwood, Inventor

By his Attorney, Herbert G. Ogle

# UNITED STATES PATENT OFFICE.

WALTER HUNNEWELL UNDERWOOD, OF NEW YORK, N. Y.

## METALLIC YARN AND FABRIC.

1,012,031.

Specification of Letters Patent. Patented Dec. 19, 1911.

Application filed November 12, 1910. Serial No. 592,004.

To all whom it may concern:

Be it known that I, WALTER H. UNDERWOOD, a citizen of the United States, and resident of the borough of Manhattan, city, county, and State of New York, have invented certain new and useful Improvements in Metallic Yarn and Fabric, of which the following is a specification.

This invention relates to an improved 10 yarn and fabric woven therefrom.

The object of the invention is to make a yarn from metallic fiber and weave the metallic yarn into a fabric.

To these ends the invention consists of the 15 improved yarn and fabric substantially as hereinafter fully described and claimed in this specification and shown in the accompanying drawings, in which:

Figure 1 is a representation of a mass of 20 metallic fibers from which the yarn is spun; Fig. 2 is a representation of a piece of yarn made from a plurality of strands spun from metallic fibers; Fig. 3 is a transverse sectional view taken through a fabric woven 25 from metallic yarn; Fig. 4 is a plan view of a portion of woven metallic fabric; Fig. 5 is a transverse sectional view of another form of fabric made from metallic yarn.

I have discovered that fine metallic fiber 30 cut or shredded from metal in the usual manner in which such material is made, or any metallic fiber having rough or serrated edges in contradistinction to smooth wires, may be spun into yarn. One form of metallic fiber suitable for spinning into a yarn is known commercially as metallic wool, and if made from steel this material is known as steel wool. The fibers of such metallic wool are ordinarily more or less irregular in cross section and the edges are serrated or roughened in the nature of wool or hair, making it possible to spin the fibers 40 into yarn.

Fig. 1 represents a mass of metallic wool 45 from which my metallic yarn may be spun, and Fig. 2 represents a compound yarn A, comprising in this instance three strands B, each of which is made from three primary strands C of metallic yarn.

Fig. 3 represents a sectional view of a 50 fabric woven from yarns D and E, and it is to be understood that the fabric may either be woven from single strands of yarn or a plurality of strands twisted, as desired.

Fig. 4 is a plan view of Fig. 3 showing 55 a simple woven fabric comprising the yarns E and D.

Fig. 5 is a transverse sectional view of 60 a fabric woven from compound yarns F and G.

The metallic wool with which I work may also be termed shredded metallic material, or if made from steel the material may be termed shredded steel. The metallic fiber may first be annealed to make it soft and 65 pliable and then spun into yarn, and after the yarn is spun or made into fabric it may be hardened, or hardened and then tempered.

The metallic yarn and fabric are useful 70 for many purposes in the arts and manufactures, for instance, when embedded in plastic material, they add very greatly to its strength and wearing qualities. The metallic fabric embedded in or combined with 75 rubber or similar material is useful for floor coverings, stair treads, packing for joints, and treads for solid and pneumatic vehicle tires. When combined with suitable material the metallic fabric makes excellent 80 surfaces for vehicle brakes, clutches and other devices requiring frictional contacting surfaces. The yarn and fabric may be made of any desired metal and when made of steel or other metals which permit of hardening 85 may be tempered to any desired degree of hardness.

The yarn may be spun from the metallic wool by carding the same, or the wool may be obtained in such form that carding is 90 unnecessary. The yarn when spun may be used as it comes from the spinning machine or it may be drawn or compressed in any suitable manner to increase the density and smoothen the surface to facilitate the weaving. If desired the metallic wool may be 95 spun or twisted together with cotton or other fiber to make a compound yarn or thread. This yarn possesses the peculiar electrical property of varying its resistance when the 100 yarn is agitated, or when placed under compression, tension or torsion, due, probably to variation in the extent of contacting surfaces of the fibers.

I claim and desire to obtain by Letters 105 Patent the following:

1. The improved yarn substantially as described spun from cut metallic fiber.

2. The improved yarn substantially as described spun from metallic fiber having serrated edges.
3. The improved yarn substantially as described spun from metallic wool.
4. The improved yarn substantially as described spun from steel wool.
5. The improved yarn substantially as described spun from shredded steel.
6. The improved yarn substantially as described spun from shredded metallic material.
7. The improved yarn substantially as described spun from annealed cut metallic fiber.
8. The improved yarn substantially as described spun from annealed metallic fiber having serrated edges.
9. The improved yarn substantially as described spun from annealed metallic wool.
10. The improved yarn substantially as described spun from annealed steel wool.
11. The improved yarn substantially as described spun from annealed shredded steel.
12. The improved yarn substantially as described spun from annealed shredded metallic material.
13. The improved tempered metallic yarn substantially as described spun from cut metallic fiber having serrated edges.
14. The improved tempered metallic yarn substantially as described spun from metallic fiber having serrated edges.
15. The improved tempered metallic yarn substantially as described spun from metallic wool.
16. The improved tempered metallic yarn substantially as described spun from steel wool.
17. The improved tempered metallic yarn substantially as described spun from shredded steel.
18. The improved tempered metallic yarn substantially as described spun from shredded metallic material.
19. The improved hardened metallic yarn substantially as described spun from cut metallic fiber.
20. The improved hardened metallic yarn substantially as described spun from metallic fiber having serrated edges.
21. As an article of manufacture, the improved fabric woven from yarn spun from metallic fibers.
22. As an article of manufacture, the improved fabric woven from yarn spun from metallic fibers having serrated edges.
23. As an article of manufacture, the improved fabric woven from yarn spun from metallic wool.
24. As an article of manufacture, the improved fabric woven from yarn spun from steel wool.
25. As an article of manufacture, the improved fabric woven from yarn spun from shredded steel.
26. As an article of manufacture, the improved fabric woven from yarn spun from shredded metallic material.

In testimony whereof I have signed this specification in the presence of two subscribing witnesses.

WALTER HUNNEWELL UNDERWOOD.

Witnesses:

K. G. LEARD,  
M. M. RIEMANN.